

Nov. 11, 1930.

E. RÜEGGER

1,781,082

ELECTRICALLY ACTUATED REFRIGERATING MACHINE

Filed May 19, 1927



## UNITED STATES PATENT OFFICE

EDUARD RÜEGGER, OF ZURICH, SWITZERLAND, ASSIGNOR TO THE FIRM AKTIENGESELLSCHAFT DER MASCHINENFABRIKEN ESCHER WYSS & CIE., OF ZURICH, SWITZERLAND

## ELECTRICALLY-ACTUATED REFRIGERATING MACHINE

Application filed May 19, 1927, Serial No. 192,648, and in Switzerland May 28, 1926.

This invention relates to partition walls or capsules for the gastight separation of rotor from stator in motors employed to operate the compressors of electrically driven refrigerating machines. As materials for the construction of such capsules, non-magnetic steel alloys having a high electrical resistance have already been employed.

As partition walls or capsules of this kind must, for constructional reasons, be made very thin, it is necessary for the material employed in their manufacture, to possess a great specific strength and strong power of resistance to corrosion and attack by acids, since the slightest rusting or the least erosion by acids renders the wall useless. The highly alloyed steels used hitherto for the manufacture of such capsules fail to satisfy the requirements above mentioned, more particularly as they are subject to molecular disintegration and consequent cracking under the influence of local attack due to atmospheric influences or the presence of acids.

The object of the present invention is to eliminate the defects aforesaid and, to this end, the capsule is made from a steel alloy containing 9 to 22% chromium, 33-5% nickel and less than 1% carbon. Such an alloy, in addition to the properties of providing satisfactory electrical conditions, being non-magnetic and possessing a relatively high electrical resistance, has also a great specific strength and great ductility as well, and it presents the further advantages of being very resistant to corrosion and attack by acids. Moreover, it can be subjected to such a heat treatment that after this treatment it does not deteriorate as might otherwise occur under certain influences (e. g. temperature, stresses arising during manufacture, electric currents and the like) in consequence of molecular disintegration. The combination of all these properties at once in the steel alloy constituted as above described tends to render it particularly suitable for the manufacture of partition walls or capsules for refrigerating machines.

Experiments have established the fact that the alloy is particularly adapted for the manufacture of capsules of the kind under

consideration if it has a nickel content of 5-9% and a chromium content of 15 to 22% or, again, a nickel content of 18 to 25% and a chromium content of 9-15% and also preferably contains about .10% of carbon, and if such alloy be subjected to an annealing process at a temperature of about 800° C.

In the accompanying drawing, which illustrates a constructional form of the invention:

Fig. 1 is a section through an electric motor driving a machine which is completely enclosed in a suitable casing and

Fig. 2 is a section through the partition wall or capsule wall, drawn to a larger scale.

The numeral 3 designates the stator of an electric motor and 2 the rotor thereof. Between these two members 2 and 3 is interposed a cap or capsule 4 serving as a partition wall. At 25 this capsule makes a gastight joint with a part 26 of a completely gastight closed housing 5 which surrounds a second housing 7. In the latter is arranged a compressor 6 swingable about trunnions 8 and driven by means of a shaft 1 by the electric motor 2, 3. This compressor 6 draws refrigerating medium from a space 19, compresses it and delivers it into a space 9 from where it flows through a pipe 10 into a chamber 11 and from there through a pipe 12 into the annular space 13 formed between the housings 5 and 7. In the annular space 13 the refrigerating medium is liquefied; the liquid refrigerating medium collects in the space 20, which is provided in its lower part with a pressure reducing device 17<sup>a</sup>. The flow of the liquid refrigerating medium to the throttling opening 17<sup>a</sup> is controlled by a float 17. The refrigerating medium expanding in the pressure reducing device 17<sup>a</sup> flows into a displacement chamber 22 which is in open connection with the evaporating chamber 23 at its lower end and by means of holes 24. The casing 15 of the evaporator is provided with ribs 16. The evaporating chamber 23 is in connection with the above-mentioned space 19 by means of a pipe 18, the part of the latter situated in the space 20 is formed as a coil 21. It is assumed that the operation of the machine will be understood from the above description of its parts without any further explanation.

The capsule 4 is made from an alloy of the constitution above stated. The interposition of a steel capsule 4 between the stator 3 and the rotor 2 of an electric-motor results in the air gap between the poles of the stator and the material of the rotor being substantially wider than in the case of a motor having no such capsule. Considerable electrical losses are introduced in consequence of this. Now since the proposed chrome-nickel-steel alloy possesses an extraordinarily great specific strength and great ductility as well, it becomes possible to make that part 4<sup>1</sup> of the capsule which is interposed between the magnet poles of the stator 2 and the material of the rotor thinner than the rest of the capsule as is shown in Fig. 2, that is to say, these other parts can be made substantially thicker. By adopting such a construction for the capsule it becomes possible to maintain a satisfactory degree of efficiency in the motor with which the device is employed.

I claim:

1. An electric motor having a rotor and a stator, a metal capsule, having a portion of reduced thickness in the air gap between the rotor and stator, said metal being a steel alloy containing 9% to 22% chromium, 33% to 5% nickel and less than 1% carbon and annealed after manufacture, of low magnetic properties, high specific strength, ductile, resistant to molecular disintegration and highly resistant to corrosion and acid attack.
2. An electric motor having a rotor and a stator, a drawn metal capsule having a portion of reduced thickness in the air gap between the rotor and stator, said metal capsule being an alloy steel containing chromium about 9% to 22%, a high nickel content of about 33% to 5% and a carbon content below 1% annealed after manufacture, having low magnetic properties, high specific strength, ductile, resistant to molecular disintegration and highly resistant to corrosion and acid attack.

In testimony whereof, I have signed my name to this specification.

EDUARD RÜEGGER.